

1,215,006.

C. A. H. DE SAULLES.  
METHOD OF TREATING ZINC BEARING MATERIALS.  
APPLICATION FILED JUNE 19, 1915.

Patented Feb. 6, 1917.

Fig 1



Fig 2



WITNESSES:

R. H. Hamilton  
G. B. Haug.

INVENTOR.

Charles A. H. de Saulles,  
BY  
Warren D. House  
His ATTORNEY.

# UNITED STATES PATENT OFFICE.

CHARLES A. H. DE SAULLES, OF NEW YORK, N. Y.

## METHOD OF TREATING ZINC-BEARING MATERIALS.

1,215,006.

Specification of Letters Patent.

Patented Feb. 6, 1917.

Application filed June 19, 1915. Serial No. 35,150.

To all whom it may concern:

Be it known that I, CHARLES A. H. DE SAULLES, a citizen of the United States, residing at New York city, in the borough of Manhattan and State of New York, have invented a certain new and useful Improvement in Methods of Treating Zinc-Bearing Materials, of which the following is a specification.

10 My invention relates to improvements in methods of treating zinc bearing material.

The object of my invention is to provide a novel method of treating zinc bearing material, such as metallic zinc or spelter, by which the capacity of production may be largely increased and by which metallic zinc dust or blue powder may be obtained in large quantities and exceeding fineness.

20 The novel features of my invention are hereinafter fully described and claimed.

In the accompanying drawing which illustrates an apparatus adapted to carry my invention into effect,

25 Figure 1 is a view partly in elevation and partly in vertical section.

Fig. 2 is a view similar to Fig. 1, the feeding funnel being removed and a ladle being shown inserted into the expansion chamber.

30 Similar reference characters designate similar parts in the different views.

1 designates a furnace of the usual type and 2 a cylindrical retort mounted therein and, preferably, having a downward and rearward inclination, whereby the molten charge 3 contained therein will have its greatest depth at the rear end of the retort.

The rear end of the retort is normally closed by a closure 4, comprising fire clay or some other suitable material, at the upper side of which is provided an opening 5 adapted to receive the small discharge end of a feed funnel 6, Fig. 1, into which molten zinc bearing material is adapted to be poured.

45 The upper end of the retort 2 is provided adjacent to its upper side with a discharge opening 7 through which zinc vapor passes into a horizontally disposed condenser 8, the discharge end of which extends into one side

50 of a vertical expansion or collecting chamber 9, preferably rectangular in cross section, and provided at its opposite side with an opening 10 adapted to be normally closed by a closure 11.

55 The lower side of the condenser 8 is preferably provided with a pocket 12, which is

adapted to receive and hold molten spelter 13, Fig. 2.

For the purpose of preventing too sudden cooling of the zinc vapor in passing through 60 the condenser 8, the condenser may be encircled by a tube 14, between which and the condenser 8 may be provided asbestos, in any suitable form, or some other suitable non-heat conducting material.

65 In the carrying of my improved method into effect, the zinc bearing material, such as metallic zinc or spelter, to be treated is poured in a molten condition into the retort 2 through the feed funnel 6. After the 70 charge has been inserted, the feed funnel is removed and the opening 5 closed by a suitable plug 16, of fire clay or other suitable material.

The furnace 1 is then fired so as to heat 75 the charge 3 of molten material to a temperature of approximately 1350 degrees centigrade.

The zinc in the charge will be vaporized and driven from the retort 2 through the 80 discharge opening 7 and into the condenser 8. The condenser 8 is retained at such a temperature, if desired, that a portion of the zinc vapor, say from 25 to 50 per cent. will be liquefied and collected in the form of 85 spelter 13 in the pocket 12 of the condenser.

The remainder of the zinc vapor will pass from the condenser into the expansion or the collecting chamber 9, in which the vapor will rapidly expand, and by reason of such 90 rapid expansion and the relatively low temperature at which the interior of the chamber 9 is retained, the larger portion of the zinc vapor which enters the chamber 9 will be precipitated therein in the form of very 95 fine zinc dust or blue powder.

From time to time the closure 11 of the expansion chamber 9 may be opened and a ladle 17 inserted through the opening 10 and under the discharge end of the condenser 8, 100 after which the molten spelter 13 in the pocket 12 of the condenser may be scraped into the ladle 17, and in such ladle removed from the apparatus.

By opening the closure 11 at suitable intervals, the temperature in the expansion chamber 9 may be retained at such a point that the zinc vapor therein will be precipitated in very fine particles.

For the purpose of removing the molten 110 lead in the charge 3, the rear closure 4 is provided at its lower side with a discharge open-

ing which is normally closed by a plug 18, Fig. 2. By removing this plug, the molten lead represented in Fig. 2 by the solid dotted lines 19 may be withdrawn by gravity. As soon as the molten lead has been removed, a plug 18 is reinserted.

An important feature of my invention consists in charging the retort 2 with zinc bearing material in a molten state. As ordinarily practised, the zinc bearing material is placed in the retort in the form of slabs or other solidified condition. In such treatment of the material, a large amount of heat is required to reduce the material to a molten state. With my improved method, the capacity of the apparatus is very much increased.

By driving the zinc vapor through the condenser 8 into the expansion chamber 9, and heating the molten charge to a temperature of approximately 1350 degrees centigrade, and then rapidly expanding the zinc vapor in the expansion chamber 9 at a relatively low temperature, much finer blue powder or zinc dust is precipitated in the expansion chamber than is obtained in the ordinary apparatus for producing zinc dust in which the condenser is eliminated and which the charge is heated to a temperature of approximately 1150 to 1200 degrees centigrade.

In the usual treatment of zinc bearing material, the retort is horizontally disposed and the material is inserted, after the removal of the rear closure in the form of slabs or solid chunks. When a new charge is to be inserted, the rear closure must be removed at intervals of 18 to 24 hours, thereby consuming time and labor, which consumption in my method is to a great extent eliminated. Furthermore the frequent removal of the rear closure effects a reduction in the temperature of the retort, thereby increasing the cost of fuel and requiring a certain length of time for the retort to become reheated to the proper vaporizing temperature. With my improved method in which the zinc bearing material is poured into the retort in a molten condition, it is unnecessary to remove the end closure, and the time required to raise the molten charge to the vaporizing temperature is much less than is required with the ordinary process just referred to.

By employing a rearwardly inclined retort having in its end closure an opening for the withdrawal of lead and other impurities, it is unnecessary in the practice of my improved method to remove the end closure, excepting at long intervals for the purpose

of removing accretions which will gradually form on the interior periphery of the retort.

I do not limit my invention to the structure herein shown and described, nor to the precise steps herein set forth, as modifications, within the scope of the appended claims, may be made without departing from the spirit of my invention.

What I claim is:—

1. The method consisting in charging a retort with molten zinc bearing material, vaporizing the zinc in the charge, and then permitting the zinc vapor to rapidly expand at a relatively low temperature to form blue powder.

2. The method consisting in charging a retort with molten zinc bearing material, vaporizing the zinc in the charge, then passing the zinc vapor through a condenser which is retained at a temperature at which a portion of the vapor will be condensed into spelter, and then permitting the remainder of the zinc vapor to be rapidly expanded at a relatively low temperature to form blue powder.

3. The method consisting in charging a retort with molten zinc bearing material, heating the charge to approximately 1350 degrees centigrade, and then permitting the zinc vapor to rapidly expand at a relatively low temperature to form blue powder.

4. The method consisting in successively charging a retort, in a continuous operation, with charges of molten zinc bearing material, vaporizing the charges, and then permitting the zinc vapor to rapidly expand at a relatively low temperature to form blue powder.

5. The method consisting in successively charging a retort, in a continuous operation, with charges of molten zinc bearing material, heating the charges to approximately 1350 degrees centigrade, and then permitting the zinc vapor to rapidly expand at a relatively low temperature to form blue powder.

6. The method consisting in successively charging a retort, in a continuous operation, with charges of molten zinc bearing material, vaporizing the charges, then passing the vapor through a condenser retained at a temperature which will permit a portion of the vapor to condense into spelter, and then permitting the remainder of the vapor to rapidly expand at a relatively low temperature to form blue powder.

In testimony whereof I have signed my name to this specification.

CHARLES A. H. DE SAULLES.